

June 21, 1932.

L. O. GRONDAHL

1,863,843

PROCESS OF PREPARING METAL FOR USE IN UNIDIRECTIONAL  
CURRENT CARRYING DEVICES  
Original Filed Jan. 7, 1925



Fig. 1.



Fig. 2.



Fig. 3.

INVENTOR:

L. O. Grondahl,  
by A. D. Venable  
His Attorney.

## UNITED STATES PATENT OFFICE

LARS O. GRONDAHL, OF PITTSBURGH, PENNSYLVANIA, ASSIGNOR TO THE UNION SWITCH & SIGNAL COMPANY, OF SWISSVALE, PENNSYLVANIA, A CORPORATION OF PENNSYLVANIA

## PROCESS OF PREPARING METAL FOR USE IN UNIDIRECTIONAL CURRENT CARRYING DEVICES

Original application filed January 7, 1925, Serial No. 1,111. Patent No. 1,640,335. Divided and this application filed July 1, 1927, Serial No. 202,811. Renewed January 15, 1932.

My invention relates to unidirectional current carrying devices, and particularly to processes of preparing metal for use in such devices.

6 The present application is a division of my copending application, Serial No. 1,111, filed January 7, 1925, for unidirectional current carrying devices, now Patent No. 1,640,335, August 25, 1927.

10 I will describe one method of preparing metal for use in unidirectional current carrying devices, and will then point out the novel features thereof in claims.

In the accompanying drawing, Fig. 1 is a 15 view showing in elevation one form of blank ready to be prepared for use in a unidirectional current carrying device in accordance with my invention. Fig. 2 is a view showing in vertical section the blank shown in Fig.

20 Fig. 1 as it appears at one point in a process embodying my invention. Fig. 3 is a view showing in vertical section a unit for use in a unidirectional current carrying device after the completion of a process embodying 25 my invention.

Similar reference characters refer to similar parts in each of the three views.

Referring to the drawing, the reference 30 character A designates a blank of suitable material, such as copper. As here shown, this blank is of circular configuration and is provided with a central aperture A<sup>1</sup>, although this particular form is not essential. In the practice of my invention this 35 blank is first cleaned; an oxide is then formed directly on the metal by oxidizing the metal at a relatively high temperature in an atmosphere containing oxygen. In the case of copper, the temperature should be in the

40 neighborhood of 1000 degrees centigrade and below the melting point of copper, such a temperature apparently being essential to the formation of a compound having the proper homogeneity, that is, non-porosity. In preparing 45 this oxide there is always formed a very thin layer of cupric oxide on the surface of the cuprous oxide which constitutes the main body of the oxide. The blank now appears as shown in Fig. 2, in which A is the copper blank, 1 is the layer of cuprous oxide,

and 2 is the coating of cupric oxide, the two oxide coatings being greatly magnified in thickness in this view. The layer of cupric oxide is removed by suitable means, such, for example, as emery cloth, as a sand blast, 55 or nitric acid. Furthermore, the layer of cuprous oxide 1 on one surface of the blank is preferably also removed, and the finished unit then has the appearance shown in Fig. 3.

In order to insure good results, the surface 60 of the copper which is to carry the cuprous oxide should be smooth and chemically clean. Some sheet copper has the appearance of having wrinkled on one side while cooling; such sheets will produce a good rectifier when the 65 smooth side is used to carry the oxide, and a poor rectifier when the wrinkled side is so used.

I have found that a unit prepared in accordance with my invention will have the 70 characteristic of offering a great deal higher resistance to the electric current flowing from the metallic copper A to the oxide 1 than the current flowing in the other direction.

The finished unit shown in Fig. 3 may be 75 utilized in the manner shown and described in my parent application, Serial No. 1,111, referred to hereinbefore.

Although I have herein shown and described only one process of preparing metal 80 for use in unidirectional current carrying devices and embodying my invention, it is understood that various changes and modifications may be made therein within the scope 85 of the appended claims without departing from the spirit and scope of my invention.

Having thus described my invention, what I claim is:

1. The process of preparing a unidirectional current carrying junction which consists in forming a smooth chemically clean surface on a copper blank, heating the blank to form oxides on said surface, and removing the cupric oxide. 90

2. The process of preparing a unidirectional current carrying junction which consists in cleaning a copper blank, heating the blank to form cuprous oxide next to the copper and cupric oxide over said cuprous oxide, and removing the cupric oxide. 95 100

3. The process of preparing a unidirectional current carrying junction which consists in heating a copper blank in the presence of oxygen to form oxides thereon, removing the oxides from a portion of the blank, and removing only the outer high resistance coating from other parts of the blank.
4. The process of preparing a unidirectional current carrying junction which consists in heating a copper blank to substantially 1000° centigrade in an oxidizing atmosphere.
5. The process of preparing a unidirectional current carrying junction which consists in heating a copper blank to substantially 1000° centigrade to form coatings of cuprous oxide and cupric oxide thereon, and removing the cupric oxide.
6. The method of obtaining a permanent rectifying junction between copper and cuprous oxide which permits substantially unobstructed flow of electrons only in the direction from the copper to the oxide, which comprises oxidizing a smooth surface of a copper body at a temperature of about 1000° C.
7. The method of obtaining a permanent rectifying junction between copper and cuprous oxide which permits substantially unobstructed flow of electrons only in the direction from the copper to the oxide, which comprises heating said copper body in an atmosphere containing oxygen to a temperature above 800° C. but below the melting temperature of copper, forming thereby on said copper a layer of cuprous oxide having an outer layer of cupric oxide.
8. The method of obtaining a permanent rectifying junction between copper and cuprous oxide which permits substantially unobstructed flow of electrons only in the direction from the copper to the oxide, which comprises heating said copper body in an atmosphere containing oxygen to a temperature above 800° C. but below the melting temperature of copper, forming thereby on said copper a layer of cuprous oxide having an outer layer of cupric oxide and removing the layer of cupric oxide.
9. The method of obtaining a permanent rectifying junction between copper and cuprous oxide which permits substantially unobstructed flow of electrons only in the direction from the copper to the oxide, which comprises heating said copper body to a temperature between 1000° and 1050° in an atmosphere containing oxygen, forming thereby on said copper a layer of cuprous oxide having an outer layer of cupric oxide.
10. In testimony whereof I affix my signature.  
LARS O. GRONDAHL.